

## UNITED STATES PATENT OFFICE

2,677,597

PROCESS OF SEPARATING SUBSTANTIALLY  
PURE  $\text{FeCl}_2$  FROM MATERIAL CONTAINING  
 $\text{FeCl}_2$  AND METALLIC COBALT

Marion Ernest Graham, Parma, and Edward A. Beidler, Columbus, Ohio, assignors, by mesne assignments, to Republic Steel Corporation, Cleveland, Ohio, a corporation of New Jersey

No Drawing. Application November 19, 1952,  
Serial No. 321,514

4 Claims. (Cl. 23—87)

1

The present invention relates to a process for the separation of ferrous chloride from material containing metallic cobalt. One embodiment of this invention is as a particular step in a large overall process for treating ores containing iron and cobalt values to obtain those values separately in some useful form.

The present application is one of a group of seven co-pending applications, all the inventions of the same inventors, four of these cases relating to nickel and reactions involving nickel and the other three relating to cobalt and reactions involving cobalt. The cases may be compared and distinguished as follows:

a. Ser. No. 160,821, filed May 8, 1950, relates to treating a starting material in the non-gaseous (liquid and/or solid) form and consisting essentially of  $\text{NiCl}_2$  and  $\text{FeCl}_2$ , and wherein there is more  $\text{FeCl}_2$  than  $\text{NiCl}_2$ . This starting material is treated in a reaction or sublimation zone, in the presence of a certain amount of metallic iron, to produce a final product which is vaporized  $\text{FeCl}_2$ , removed from the sublimation zone as such, leaving only metallic iron and metallic nickel in the sublimation zone.

b. Ser. No. 210,433, filed February 10, 1951, relates to treating a starting material, essentially the same as Ser. No. 160,821, except that in this instance the starting material is introduced into the reaction zone in a solely gaseous state. The reaction and the final products are substantially the same as in Ser. No. 160,821.

c. Ser. No. 160,822, filed May 8, 1950, relates to the preventing or minimizing of a possible back reaction. The starting material consists essentially of ferrous chloride and metallic nickel. It is desired to separate these materials without permitting, or at least minimizing, a possible back reaction therebetween which would produce nickel chloride and metallic iron. To do this, the starting material is introduced into a reaction or sublimation zone in which metallic iron is present. The starting material as introduced into this zone is in a non-gaseous state. The final products are substantially pure ferrous chloride vapor, which is removed from the zone as such, and metallic nickel and metallic iron which remain in the zone.

d. Ser. No. 294,058, filed June 17, 1952, discloses a process for treating a starting material substantially the same as in Ser. No. 160,821. This case has been amended so as to preclude the claims reading upon separation of the products of the reaction by vaporization as in Ser. No. 160,821; but in this case the separation following the reaction is effected by withdrawing the me-

2

tallic nickel produced (by a reaction the same as in Ser. No. 160,821) by withdrawing massive pieces of iron, to which the deposited nickel adheres physically, from the fused bath of the starting materials. Neither the ferrous chloride nor any nickel chloride present is intentionally volatilized. This application is junior to application Ser. No. 160,821, so that the only subject matter claimable therein is subject matter which cannot be supported by the disclosure of Ser. No. 160,821; all the common subject matter being claimed in Ser. No. 160,821.

e. Ser. No. 291,816, filed June 4, 1952 is the first of the three cobalt applications and is the cobalt counterpart of the nickel case, Ser. No. 160,821, distinguishing therefrom by being directed to cobalt and its chloride, rather than nickel and its respective chloride. This case is further distinguished in the degree of purity of the sublimate.

f. Ser. No. 320,835, filed November 15, 1952, is the cobalt counterpart of nickel case, Ser. No. 210,433. It distinguishes from cobalt case Ser. No. 291,816 in the same way discussed above as to the respectively corresponding nickel cases, while distinguishing from its corresponding nickel case, Ser. No. 210,433, by the differences between cobalt and nickel.

g. Ser. No. 321,514, filed November 19, 1952 (the present application), is the cobalt case corresponding to the nickel case Ser. No. 160,822. It distinguishes from the other cobalt cases as discussed above in respect to the respectively corresponding nickel cases, while distinguishing from its nickel counterpart, Ser. No. 160,822, by the differences between nickel and cobalt.

One of the early phases of an overall process in which the present invention could serve as a particular step, could, for example, be the chloridizing of that part of an original iron-nickel-cobalt ore material from which the nickel values had been removed, as by a selective precipitation step. If such a chloridizing step, which forms no part of the present invention, be carried out under conditions such that the iron values are selectively chloridized, while the cobalt values are reduced to metallic cobalt, there would be produced a material containing  $\text{FeCl}_2$ , metallic cobalt, usually in finely divided form, gangue and possibly, in addition, some reduced metallic iron. It is such a mixture that is contemplated as the starting material for the process of the present invention. It will be understood, of course, that such a material may be the result of other processes and that the method of producing the aforesaid mixture forms no part of this invention.

It is known that ferrous chloride can be vaporized and thereby separated from inert materials under suitable temperature conditions. However, we have found that when metallic cobalt is present, mixed with ferrous chloride, a back reaction tends to take place between some of the metallic cobalt and the ferrous chloride present to form metallic iron and cobalt chloride. This reaction may be represented by the equation:



As will be more particularly pointed out in the specific examples hereinafter given, the tendency of this reaction to proceed from left to right is more pronounced, the higher the ratio of  $\text{FeCl}_2$  to metallic cobalt. It will be seen that the occurrence of such reaction is undesirable for several reasons: first, the sublimed material will not consist of substantially pure ferrous chloride as desired, but will be contaminated with cobalt chloride; and, second, at least some of the cobalt, which may be desired to be recovered in the metallic state, is converted to a volatile chloride and lost or mixed with the ferrous chloride.

A general object of the present invention is, therefore, to provide a method of separating ferrous chloride from the remaining materials in the form of substantially pure ferrous chloride, containing not over about 1% by weight of cobalt chloride and preferably substantially less, as an impurity.

It is a further object to maintain the metallic cobalt in the starting material in metallic form, while minimizing the amount that will be lost as volatile cobalt chloride.

Summarizing the present invention, the separation of ferrous chloride containing less than about 1% cobalt chloride by weight as impurity is accomplished by providing in the starting material an amount of metallic iron at least equal to the weight of the metallic cobalt therein. The metallic iron may be all or in part present in the original mixture, or it may be entirely added. The term "providing metallic iron" or equivalent language, as used in the claims, includes either a starting material which has such metallic iron present initially, or a starting material which had no, or too little, initial content of metallic iron, but to which metallic iron has been added to the extent necessary, in accordance with the present invention. The material, which now includes ferrous chloride, metallic cobalt, metallic iron and possibly some inert or gangue materials, is then heated to a temperature in the range of about 600° C. to about the boiling point of  $\text{FeCl}_2$  at the prevailing pressure for a time sufficient to vaporize the  $\text{FeCl}_2$  present.  $\text{FeCl}_2$  boils at about 1025° C. at 760 mm. pressure. Vaporized  $\text{FeCl}_2$  may, if desired, be removed from the non-volatile material by a sweep gas. As it has been found that the equation given above, as illustrating a reaction which is to be inhibited or at least minimized in accordance with the present invention, is a reversible one which tends to reach an intermediate equilibrium condition, the present invention provides conditions assuring the desired results. Thus, by providing a quantity of finely divided iron in the material as aforesaid, there is assured either of the following results: (a) that the equation will operate in the direction shown only to a very limited extent and will produce only a small amount of  $\text{CoCl}_2$ , or, (b) substantially all of such  $\text{CoCl}_2$  as may be formed will immediately react with metallic iron, present as

aforesaid, to produce metallic cobalt and  $\text{FeCl}_2$ . The net result is that by far the greater part of the metallic cobalt initially present remains as such in the non-volatile residue after all the  $\text{FeCl}_2$  initially present has been sublimed or distilled therefrom.

Thus, in accordance with the present invention, it is necessary to have present metallic iron to react with any cobalt chloride which may be formed from a reaction between the metallic cobalt and the ferrous chloride originally present. We have found that when using an amount of iron at least equal to the weight of the metallic cobalt present, the amount of cobalt chloride which is formed and carried over to the sublimate is reduced to such an extent that the ferrous chloride in the sublimate contains less than 1% by weight of cobalt chloride as an impurity. We have further found that if the iron is present in a ratio of about five parts by weight to about one part by weight of metallic cobalt, the sublimate obtained from heating such a material to a temperature where  $\text{FeCl}_2$  has a substantial vapor pressure, will be  $\text{FeCl}_2$  containing less than about 0.2%  $\text{CoCl}_2$  as an impurity. It is our conclusion that when a 5:1 ratio of iron to cobalt is used, such sublimate is for all practical purposes, substantially free of cobalt chloride. However, sublimate containing even smaller amounts of cobalt chloride as an impurity, may be obtained by the use of an amount of iron in excess of the amount needed to produce a 5:1 by weight ratio in respect to cobalt, as set forth in detail in the specific examples which follow. Such conditions are undesirable only to the extent that they reduce the purity of the metallic cobalt left as a residue after the  $\text{FeCl}_2$  has been removed.

As has been indicated above, the metallic iron which serves to inhibit as to minimize the formation and/or separation by sublimation from the mass of volatile cobalt chloride and thereby serves to minimize the loss of cobalt in volatile form, may be initially present in the material in sufficient quantity to produce this effect, or it may be wholly or partially added.

In view of the fact that a chemical reaction, involving the metallic iron, may be called for, in accordance with the present invention, as aforesaid, it is desired to have the iron present in a readily available form. For this reason the iron is preferably present and/or is introduced in a finely divided form and is well mixed with the other solid and/or liquid ingredients of the starting materials.

While we have found that the tendency of the reaction between ferrous chloride and metallic cobalt to form cobalt chloride and metallic iron is more pronounced as the ratio of ferrous chloride to metallic cobalt in the starting material increases, the purity of the sublimate with respect to the amount of cobalt chloride contained therein as an impurity, can be controlled by the addition of metallic iron to an extent that is substantially independent of the ratio of  $\text{FeCl}_2$  to metallic cobalt in the starting material. This is amply demonstrated by actual examples of the present process hereinafter given.

In practicing the present invention, it is necessary to produce ferrous chloride vapor, so that the material being treated must be held in a temperature range sufficiently high to insure that the ferrous chloride will have a sufficient vapor pressure. The low limit of such a temperature range may be conveniently placed at about 600°

C., at which temperature  $\text{FeCl}_2$  has a substantial vapor pressure. It has been found, in practice, that at temperatures below about  $600^\circ \text{C}$ , the rate of vaporization of  $\text{FeCl}_2$  is so slow as to make the process impractical. The upper limit of the temperature range is fixed by the boiling point of ferrous chloride, which, at standard atmospheric pressure, is about  $1025^\circ \text{C}$ . In view of the fact that the volatilization of the ferrous chloride is an endothermic process, the temperature of the mass from which the  $\text{FeCl}_2$  is volatilized cannot exceed this boiling point as long as any substantial amount of ferrous chloride remains therein. However, it will be understood that in cases where the materials are maintained at super-atmospheric pressures, the boiling point of ferrous chloride will be higher, so that correspondingly higher temperature limits can be employed. Therefore, the upper limit of the temperature range may be the boiling point of ferrous chloride at whatever pressure is being employed.

In general, it may be said that while the temperature is not particularly critical, the rate of removal of the ferrous chloride from the material present is, of course, a function of the temperature, so that the process is completely operative throughout a large temperature range as stated, the rate differing with different temperatures. The removal of vaporized ferrous chloride from the system may be effected either by operating at the boiling point of ferrous chloride or by using a sweep gas in a manner similar to a steam distillation. Such a sweep gas is preferably an inert gas, such as nitrogen.

It is contemplated that the process of the present invention may be carried on either as a batch or as a continuous type operation, suitable or conventional apparatus, per se forming no part of the present invention, being used in either case. The  $\text{FeCl}_2$  vapor, which is produced as a result of this process, may be condensed to solid or liquid form by any suitable means and may be used for any desired purpose. Alternatively, the vapor may be maintained at its high temperature and used for any purpose to which  $\text{FeCl}_2$  vapor is adapted. The residual material will contain metallic iron and metallic cobalt. These metals may be separated from the gangue by any suitable method, magnetic or otherwise, and/or melted together to form an alloy.

The following examples illustrate the present process:

#### EXAMPLE I

To illustrate the extent to which metallic cobalt and ferrous chloride react in the absence of metallic iron to produce volatile cobalt chloride and with different ratios of  $\text{FeCl}_2$  to cobalt, reference is made to Table I below. The results set forth in this table illustrate the amount of metallic cobalt that is converted to volatile cobalt chloride as a result of heating mixtures consisting of different amounts of ferrous chloride and metallic cobalt at  $1000^\circ \text{C}$ . in an atmosphere of nitrogen for one hour.

Table I

| Weight Ratio of Ferrous Chloride to Metallic Cobalt | Percent of Metallic Cobalt Converted to Volatile $\text{CoCl}_2$ | Cobalt Chloride Content of Ferrous Chloride Sublimate in percent |
|-----------------------------------------------------|------------------------------------------------------------------|------------------------------------------------------------------|
| 880                                                 | 54                                                               | 0.14                                                             |
| 88                                                  | 39                                                               | 1.00                                                             |
| 1                                                   | 9                                                                | 20.10                                                            |

Thus it is seen that without the presence of metallic iron a very substantial portion of the metallic cobalt present in mixtures of ferrous chloride and metallic cobalt is converted to volatile cobalt chloride. It will be further seen that greater percentages of metallic cobalt are so converted in mixtures where the ratio of ferrous chloride to metallic cobalt is high than in which this ratio is relatively low.

#### EXAMPLE II

The effect of the addition of varying amounts of metallic iron on the purity of the ferrous chloride obtained and the percent of cobalt converted to the chloride is illustrated by the results set forth in Table II below. The results set forth in this table were obtained by treating mixtures containing ferrous chloride and metallic cobalt, in all instances in the weight ratio of 88 parts of ferrous chloride to 1 part of metallic cobalt, at  $1000^\circ \text{C}$ . for about one hour in a stream of nitrogen.

Table II

| Ratio of Metallic Iron added to Metallic Cobalt | Percent of Metallic Cobalt converted to Volatile $\text{CoCl}_2$ | Cobalt Chloride Content of Ferrous Chloride Sublimate in percent |
|-------------------------------------------------|------------------------------------------------------------------|------------------------------------------------------------------|
| 1:9                                             | 44                                                               | 1.14                                                             |
| 3:9                                             | 40                                                               | 1.04                                                             |
| 1:1                                             | 31                                                               | 0.79                                                             |
| 2:1                                             | 21                                                               | 0.53                                                             |
| 3:1                                             | 13                                                               | 0.33                                                             |
| 5:1                                             | 7.1                                                              | 0.18                                                             |
| 20:1                                            | 2.8                                                              | 0.072                                                            |

Thus it is seen that as greater amounts of metallic iron are provided, the purity of the ferrous chloride sublimate may be increased, although it has not been found possible to eliminate entirely the presence of cobalt chloride as an impurity in the sublimate.

#### EXAMPLE III

The results set forth in Table III below illustrate that the purity of the ferrous chloride sublimate can be controlled as to its content of cobalt chloride by the addition of varying amounts of metallic iron; and that this purity is controlled by the ratio of metallic iron provided to metallic cobalt originally present in the mixture, rather than by the ratio of ferrous chloride to metallic cobalt originally present. The results set forth in this series of tests were obtained by treating a mixture consisting of ferrous chloride and metallic cobalt, always in the weight ratio of 8.8 parts of ferrous chloride per part of metallic cobalt, at  $1000^\circ \text{C}$ . in a current of nitrogen for about one hour.

Table III

| Ratio of Metallic Iron added to Metallic Cobalt | Percent of Metallic Cobalt converted to Volatile $\text{CoCl}_2$ | Cobalt Chloride Content of Ferrous Chloride Sublimate in percent |
|-------------------------------------------------|------------------------------------------------------------------|------------------------------------------------------------------|
| 3:4                                             | 5.78                                                             | 1.48                                                             |
| 1:1                                             | 3.42                                                             | 0.86                                                             |
| 2:1                                             | 1.47                                                             | 0.37                                                             |
| 5:1                                             | 0.72                                                             | 0.18                                                             |

This example, taken in conjunction with Example II above, illustrates that ferrous chloride containing less than 1% of cobalt chloride as an impurity, may be obtained by providing in the starting material an amount of metallic iron at least equal to the weight of the metallic cobalt

therein, no matter what ratio of ferrous chloride to metallic cobalt is originally present and also that a pure ferrous chloride product containing less than 0.2%  $\text{CoCl}_2$  by weight may be obtained in all cases by providing sufficient metallic iron to equal at least five times the weight of the metallic cobalt present in the starting material.

While it is desirable to obtain as pure a product as possible in terms of ferrous chloride, additions of large amounts of metallic iron will obviously result in the formation of a non-volatile residue which is progressively less rich in metallic cobalt as the amount of metallic iron added is increased.

While we have described our process in general and have set forth in some detail the chemical and physical requirements thereof, it is recognized that the process may be operated by the substitution of such equivalents as will suggest themselves to those skilled in the art from the foregoing disclosure. We do not wish to be limited, therefore, except by the scope of the appended claims, which are to be construed validly as broadly as the state of the art permits.

What is claimed is:

1. The process of separating ferrous chloride from a starting material consisting essentially of  $\text{FeCl}_2$  and metallic cobalt, while substantially preventing loss of cobalt in the form of  $\text{CoCl}_2$ , which comprises introducing said starting material in a non-gaseous state into a sublimation zone, providing in contact with said material in said sublimation zone sufficient metallic iron to assure that such iron is present in an amount at least equal to the weight of the metallic cobalt in said starting material which is in said zone, maintaining said material in said zone including said me-

tallic iron within the temperature range of about 600° C. up to the boiling point of  $\text{FeCl}_2$  at the ambient pressure, vaporizing all the  $\text{FeCl}_2$  present, and separating the volatilized  $\text{FeCl}_2$  containing less than about 1%  $\text{CoCl}_2$  by weight from the remainder of said material by passing the volatilized  $\text{FeCl}_2$  from said zone to leave solely metallic iron and cobalt in said zone.

2. The process according to claim 1, in which said metallic iron is present in said zone in a weight ratio to metallic cobalt of at least about 5:1, the  $\text{FeCl}_2$  vapor so separated containing less than about 0.2%  $\text{CoCl}_2$  by weight.

3. The process according to claim 1, in which said material including said metallic iron is maintained at a temperature of about 1000° C.

4. The process in accordance with claim 1, in which said metallic iron in said reaction zone is in a finely divided condition, and in which the step of removing said volatilized  $\text{FeCl}_2$  from said zone is assisted by passing an inert gas through said zone to serve as a sweep gas.

#### References Cited in the file of this patent

#### UNITED STATES PATENTS

| Number    | Name  | Date          |
|-----------|-------|---------------|
| 2,396,792 | Kroll | Mar. 19, 1946 |

#### OTHER REFERENCES

J. W. Mellor: *Modern Inorganic Chemistry*, pages 432, 433; new impression of 8th ed., January 1935, Longmans, Green and Co., N. Y.

Lewis: "An Outline of First Year College Chem." (1945 ed.), pages 48-50. Barnes and Noble Inc., N. Y.